

June 4, 1940.

R. PERRIN

2,203,179

PROCESS FOR THE MANUFACTURE OF HEMATITE CAST IRON

Filed March 14, 1938



Inventor:

Rene Perrin  
by his Atty.  
Stibbins, Blank & Parmelee

## UNITED STATES PATENT OFFICE

2,203,179

PROCESS FOR THE MANUFACTURE OF  
HEMATITE CAST IRON

René Perrin, Paris, France, assignor to Societe d'Electrochimie, d'Electrometallurgie et des Acieries Electriques d'Ugine, Paris, France, a corporation of France

Application March 14, 1938, Serial No. 195,842  
In France March 16, 1937

4 Claims. (Cl. 75—48)

It has already been proposed to make hematite cast iron by means of the Thomas converter starting from cast iron containing phosphorus by first transforming this cast iron into a dephosphorised steel and by then recarburising this steel by addition of carbon. The recarburisation may be effected either in the converter itself or by successive turning down of the converter with very short blowings or in a ladle by transfer.

In the same process it has been proposed to add to the metal during the recarburisation additions of materials producing evolution of heat in order to increase the solubility of the carbon.

By the present invention I have discovered the means of effecting this recarburisation in conditions such that:

1. The solution of the carbon is extremely rapid.

2. The addition of materials giving off heat to obtain an increase of the solubility of the carbon is in no way necessary.

3. The operation is very simple and the heat losses are very small.

4. The operation leads to high yields of the recarburising material and moreover yields which are extremely regular from one operation to another.

5. The final composition of the cast iron obtained is extremely regular from one operation to another.

In order to arrive at these results I propose to submit the material to be recarburised—generally extra mild steel coming from the converter—and the recarburising material—for example coke or charcoal—to successive energetic intermixings repeated at short intervals in an apparatus formed for example of two chambers arranged so as to permit with rapid frequency the contents of one of the chambers to be poured into the other and reciprocally with a force sufficient to bring, during the pourings thus effected, the carboniferous elements below the surface of the metal producing strong eddies.

Such an apparatus may be formed in particular of two chambers opposing mouth to mouth and each to some extent forming an extension of the other. The assembly of the two chambers is animated with an oscillating or rotating movement, the liquid steel and the carbon which it is desired to react are introduced into the apparatus and this is subjected to a series of successive oscillations or rotations which project the steel and carbon from one chamber into the other reciprocally. The ratio between the volume of

each chamber and the charge of metal and solid reacting substance which is introduced therein for treatment is so chosen that the height of fall of the said charge from one chamber into the other is sufficient for the carboniferous substance to be entrained into the body of the metal and to produce strong eddies.

It is important however to explain how these successive pourings should be effected for the success of the operation. If it is presumed that one of the chambers of the apparatus contains liquid steel upon which for example pieces of coke have been dropped and that the metal from this chamber is poured slowly into the other chamber of the apparatus, the coke having a density much less than that of the metal will remain at the surface of the bath and only a very slow reaction and solution will be produced.

If on the contrary the metal is poured with force, strong eddies will be produced, the whole or a large part of the coke is entrained into the body of the metal and experiment then shows that the speed of the reactions and of the solution increases to a very considerable extent as well as the regularity of the results obtained.

It is this phenomenon of entrainment of the coke into the body of the metal which is to be sought, this entrainment is moreover also facilitated by the eddies which are produced by the shock of the molten metal against the walls.

It is important in all cases that the pouring of the metal with the carboniferous substance should be sufficiently strong for there to be penetration of the pieces of the carburising material into the body of the metal which condition is the more difficult to produce the greater the difference between the density of this material and that of the metal. This result may be obtained in the most simple way for example in the type of apparatus described below. At each oscillation rapid pouring is produced with interpenetration of the phases present. At the end of a certain number of operations recarburation is effected.

The greater the force of the pourings the more rapid the carburation all other things being equal.

In a general way the pouring should be effected with as much force and rapidity as possible compatible with good durability of the refractories and of the apparatus.

However in general the reaction between the molten metal and the recarburising material will give rise to considerable evolution of carbon monoxide particularly at the beginning of the

operation in the case when one starts from an extra mild Thomas steel which is strongly oxidised. In this case precautions should be taken so that the rapidity of the reaction is not such that it leads to an explosion or even to expulsion of metal out of the apparatus.

Apart from the fact that the apparatus should be open to permit the outlet of the gases as they are formed, two means may be employed to regulate the rapidity of the reaction.

1. The successive pourings may be slowed down. But in this case the pouring must remain sufficiently strong for there to be penetration of the carboniferous material into the body of the molten metal which condition is essential for rapid reaction.

2. The quantities of carboniferous material may be introduced periodically by fractions in regulated proportions (at each pouring for example) or even in a less divided form. It is important not to use too fine powder which may be partially taken away by the gases which are evolved.

The adjustment will be effected for each particular treatment by previous tests.

It will be observed when operating under the conditions described above that in a very short time even when starting from an extra mild steel a cast iron having the desired carbon content will be obtained.

The starting materials to be utilised for re-carburation may be coke, charcoal, anthracite or any other carboniferous material capable of dissolving in the metal. They will be chosen as free from sulphur as possible.

Although the addition of substances giving off heat is not necessary to effect the dissolution of the carbon substances may if desired be introduced such as silicon or manganese or other alloying elements with the object of bringing the cast iron to the desired composition.

The process of the invention is capable of being applied in advantageous conditions in an apparatus such as that shown schematically by way of example in the accompanying drawing.

The apparatus comprises two chambers 1 and 2, relatively deep, connected to one another by their mouth and communicating with a medial aperture 3 open to the atmosphere. These two chambers are constituted by a metallic casing 4 provided with a refractory lining 5. The whole is mounted upon a shaft 6 capable of turning in support bearings 7 and receives an alternating oscillatory movement by means of a driving mechanism of suitable known type which is not shown. This movement brings turn by turn the chambers 1 and 2 into a position respectively high or low and with a strong inclination which causes its contents to be projected strongly and from as great a height as possible into the other chamber. This effect may be facilitated by giving at first to the apparatus a speed sufficient for centrifugal force to maintain or tend to maintain the charge towards the bottom of the chamber which contains it and then by causing this speed to diminish rapidly, when the bottom of the chamber is about to reach or has reached the top of its course.

#### *Example of operation*

Into the apparatus 3 metric tons of extra mild strongly oxidised steel were introduced. The carbon content of this steel was 0.05%, the phosphorus content 0.010%. 65 kgs. of coke with a low sulphur content were added.

To the apparatus a series of oscillations were imparted. An intense ebullition occurred due to the action of the coke on the oxides present in the metal. The ebullition slowed down as the oscillations continued. After six oscillations 65 kgs. of coke were added.

At the end of 12 oscillations in all the operation was terminated. The cast iron obtained contained: C=3.5%; P=0.012%; S=0.025%.

The melting point of the final metal being 10 notably lower than that of the initial metal, according to the invention the heat which has become available in consequence of the differences in temperature in question may be utilised to increase finally without expenditure of external 15 heat or without necessarily having to develop internal heat, the weight of the initial metal and this without modifying substantially its composition or by modifying it in the sense of an addition of alloying elements. For this purpose to the 20 bath of metal is added either during the operation of treatment by the solid material or at the end of the operation, that is to say when the transformation of the initial metal is finished, pieces, fragments or scraps of metal or alloy. 25 Due to the fact that the metallic bath is at a temperature above its melting point and due likewise to the speed of the successive pourings, the elements thus added dissolve rapidly in the bath even if they are introduced cold, and this without the bath cooling below the temperature which should be maintained for its subsequent use.

There is obtained finally by recovery of the excess heat which otherwise would be lost a weight of metal above that of the initial metal 35 increased by that of the solid reacting material which has passed into the metal, for example if the manufacture of cast iron is concerned, a weight of cast iron above that of the initial steel increased by that of the carbon which has passed 40 into the cast iron.

The proportion of the pieces or fragments of metal or of scrap or of alloying elements which it is possible to incorporate thus in the bath of metal is considerable and may reach practically 45 5% and even more of the initial weight of the metal, but it is naturally limited by the quantity of excess heat available in the cycle. It depends also on the state of division in which are the materials to be melted, for example fine scrap 50 metal or scrap iron or turnings will be capable of dissolving very rapidly. This proportion may readily be determined in each case by calculation or even better by experiment. The importance of such metallic additions in the special 55 apparatus employed resides in the particularly economical utilisation which is thus made of these materials and of the excess heat, which materials are utilised normally by fusion in the electric or Martin furnace, that is to say with 60 expenditure of external heat.

What I claim is:

1. The process of making cast iron, which comprises subjecting molten mild steel and solid re-carburizing material simultaneously to a series of successive rapid pourings which are effected with a force sufficient to insure during these pourings an intimate and turbulent mixture of the metal and re-carburizing material, and during or at the end of the carburizing reaction adding solid 70 metallic or alloying elements which are caused to dissolve by means of the heat rendered available by reason of the difference of the melting point of the initial metal and that of the re-carburized metal.

2. The process of making cast iron, which comprises subjecting molten mild steel and solid re-carburizing material simultaneously to a series of successive rapid pourings which are effected with a force sufficient to insure during these pourings an intimate and turbulent mixture of the metal and re-carburizing material, and dissolving solid metallic or alloying elements in the bath which has been at least partially carburized and without the supply of external heat to the bath.
3. The process of making cast iron, which comprises subjecting molten mild steel and solid re-carburizing material simultaneously to a series of successive rapid pourings which are effected with a force sufficient to insure during these pourings an intimate and turbulent mixture of the metal and re-carburizing material, and continuing the pourings until the carbon content of the bath is raised by an amount of the order of at least 3.0%, and dissolving solid metallic or alloying ele-
- ments in the bath which has been at least partially carburized and without the supply of external heat to the bath.
4. The process of making cast iron, which comprises subjecting molten mild steel and solid re-carburizing material simultaneously to a series of successive rapid pourings which are effected with a force sufficient to insure during these pourings an intimate and turbulent mixture of the metal and re-carburizing material, and continuing the pourings until the carbon content of the bath is raised by an amount of the order of at least 3.0%, and dissolving solid metallic or alloying elements in the bath which has been at least partially carburized and without the supply of external heat to the bath, the mild steel being substantially free from sulphur and the carburizing reaction being carried out in the absence of added oxidizing agents.

RENE PERRIN. 20